

Feb. 3, 1948.

E. C. PFEFFER, JR., ET AL

2,435,509

STITCHLESS SHIRT COLLAR AND METHOD OF MAKING IT

Filed Dec. 27, 1943

2 Sheets-Sheet 1



Inventors  
Edward C. Pfeffer, Jr.  
Laurence M. Miller  
by Robert Cushman Greene  
Attys.

Feb. 3, 1948.

E. C. PFEFFER, JR., ET AL

2,435,509

STITCHLESS SHIRT COLLAR AND METHOD OF MAKING IT

Filed Dec. 27, 1943

2 Sheets-Sheet 2



Inventors  
Edward C. Pfeffer Jr.  
Laurence M. Miller  
by Robert C. Cramer  
Atty's.

## UNITED STATES PATENT OFFICE

2,435,509

STITCHLESS SHIRT COLLAR AND METHOD  
OF MAKING IT

Edward C. Pfeffer, Jr., Troy, and Laurence M. Miller, Albany, N. Y., assignors to Cluett, Peabody & Co., Inc., Troy, N. Y., a corporation of New York

Application December 27, 1943, Serial No. 515,690

3 Claims. (Cl. 2—143)

1

This invention pertains to seams for uniting textile fabrics or the like and to a novel method of making such seams, more particularly to a flexible seam in which the usual stitches are replaced by adhesive. While of general utility, the invention is here more particularly described and illustrated by way of example but without limitation in its application to certain specific forms of seam, and to the manufacture of shirt collars and shirts.

Heretofore the customary way of uniting the constituent parts of a garment, for instance a shirt collar, has been by sewing them together. Stitched seams provide a satisfactory flexible union between such parts but involve the use of a sewing machine; sewing thread which is an expensive material and which tends to produce puckers or wrinkles at the location of the seam; and the employment of a skilled operator in order to attain the speed and accuracy requisite in commercial production; and the completed seam, no matter how carefully formed, shows as a distinct line emphasized by the needle holes in the finished article.

In accordance with the present invention, a durable, flexible, smooth and wrinkleless seam may be formed without the employment of a sewing machine and by operators relatively unskilled, but without sacrifice of speed, and the completed article is unmarred by any appreciable line or visible change in surface appearance at the location of the seam.

In general, this novel seam involves the employment of a narrow, flexible tape of a thermoplastic material, for example a synthetic resin, which is interposed between the plies of fabric which are to be joined and which, when subjected to heat and pressure, fuses and thus permanently joins the fabric plies.

In the accompanying drawing, wherein certain desirable steps in the process of forming such seams and garments comprising seams of this type are illustrated by way of example,

Fig. 1 is a plan view of a completed collar made in accordance with the present invention;

Fig. 2 is a plan view of a fabric blank useful in forming the facing or outer ply of the collar;

Fig. 3 is a plan view of a lining blank having adhesive tape applied to its margins in preparation for folding;

Fig. 4 is a similar view of a blank designed to form the back ply of the collar, this blank also having adhesive tape on its margin;

Fig. 5 is a section on the line 5—5 of Fig. 3;

Fig. 6 is a section on the line 6—6 of Fig. 2;

2

Fig. 7 is a section on the line 7—7 of Fig. 4;

Fig. 8 is a section to large scale illustrating the proper relative arrangement of the front, back and lining blanks in assembling them;

5 Fig. 9 is a view similar to Fig. 8 but showing the first step in the folding of the united blanks;

Fig. 10 is a section to large scale on the line 10—10 of Fig. 11;

Fig. 11 is a front elevation of the collar after 10 turning but showing the constituent plies separated along the top edge of the collar, and showing adhesive tape interposed between the separated plies;

Fig. 12 is a plan view of a neckband blank with 15 a tape along one margin;

Fig. 13 is a section to large scale through the top edge portion of the collar with the neckband blanks united thereto;

Fig. 14 is a similar view showing the neckband 20 blanks after turning;

Fig. 15 is a plan view to large scale showing one end of the collar with the neckband attached but with the front and rear plies of the neckband turned up;

25 Fig. 16 is a view similar to Fig. 15 but showing the neckband plies turned down;

Fig. 17 is a section illustrating one way of forming an adhesive seam uniting two plies of fabric;

Fig. 18 illustrates another way of forming a 30 seam; and

Figs. 19 and 20 are sections illustrating still further ways of forming seams uniting fabric plies.

Referring to the drawings, the collar top is 35 indicated at 1 and the neckband portion at 2. The collar top comprises three plies, the facing ply blank being indicated at 3 (Fig. 2), the lining blank at 4 (Fig. 3), and the rear ply or back blank at 5 (Fig. 4). These blanks may be formed from

40 any usual material (for example woven cotton broadcloth) employed for the purpose, and may be cut to the proper shape in the usual way. In accordance with the present invention, the lower edge (upper edge as shown in the drawing) and

45 the ends of the lining blank 4 are provided with a narrow band 6 of adhesive. This band 6 is preferably provided as a narrow tape or ribbon, for example approximately  $\frac{1}{8}$ " wide and of the order of 0.004" thick, consisting of a thermoplastic resin. The resin selected may, for example,

50 be a vinyl acetate-vinyl chloride copolymer plasticized by the incorporation of a suitable plasticizer. For instance, the tape or ribbon may consist of 68 parts vinyl acetate-vinyl chloride copolymer, plasticized with 38 parts of di-(2-

ethyl hexyl) phthalate. The percentage of plasticizer may be varied from 20 to 40% based on the weight of the resin, and largely depends upon the molecular weight of the superpolymer being used and the degree of stiffness desired. Other thermoplastic resins besides the vinyl copolymer may be used. Excellent results are thus obtained with Saran (polyvinylidene chloride), polyvinyl butyral and nylons (polyamides).

Whatever the thermoplastic resin which is selected, it must be very flexible and capable of withstanding the heat and pressure in forming the bond between the fabric parts without discoloration or other unfavorable affects; it must be colorless and substantially unaffected by washing fluids or the temperature encountered in washing; it must be capable of withstanding ironing operations without discoloration or becoming so soft that the seam pulls apart during ironing; it must provide a seam strong enough to meet the requirements of the garment manufacturer, and the seam when formed must not be unduly stiff. To avoid undue stiffness and any danger that the resin may be in sufficient amount to strike through the fabric, but at the same time providing sufficient bond, it appears that the thickness of this tape should not be less than 0.002" nor more than 0.008", preferably about 0.004".

Having prepared the thermoplastic tape as above suggested, this tape is laid along the edges of the lining blank, as above stated, and is calendered to the blank so as to adhere to the latter. The rear or back blank of the collar top is likewise provided with a marginal band 7 of the thermoplastic material. Having prepared the blanks 3, 4 and 5, and having provided the blanks 4 and 5 with these marginal adhesive tapes, the blanks are assembled as shown in Fig. 8 with the facing blank 3 interposed between the lining and rear blanks and with the adhesive tapes 6 and 7 disposed in contact with the facing blank 3. The marginal portions of the blanks are now subjected to heat and pressure such as to cause the adhesive to bond the blanks together along a narrow marginal area of a width substantially corresponding to the width of the tape. Temperatures of the order of from 400° to 500° F. are suitable for the purpose, and a pressure of the order of 133 lbs. per square inch applied for a period of from 1 to 3 seconds is sufficient to provide the desired intimate bond between the plies.

The points of the collar are now preferably trimmed, the collar is turned in accordance with usual practice, and the collar points are formed, all in substantially the same manner as though the blanks had been united by a sewed seam.

The top edges of the blanks are now trimmed, and a length 8 (Figs. 11 and 13) of the thermoplastic tape is now interposed between the facing blank 3 and the lining blank 4 at the top edge (lower edge as shown in Fig. 11) of the collar top, and a similar tape 9 is interposed between the lining blank 4 and the rear or back blank 5. Preferably this tape 9 is sufficiently longer than the top edges of the blanks so as to provide extensions 9a (Figs. 15 and 16) projecting beyond the ends of the collar top. Preferably the tape 9 may be somewhat wider than the other tapes, for example it may be of a width of  $\frac{1}{8}$ ", and the extensions 9a may be of a length approximating  $\frac{1}{2}$ " beyond the end edges of the collar top. Having interposed the tapes 8 and 9 between the edges of the blanks, the parts are subjected to

heat and pressure so as to bond the top edges of the collar top together.

Neckband blanks 11 and 12 (Figs. 12, 13 and 14) are provided, such blanks being of the usual size and shape and cut from usual materials (for example woven cotton broadcloth), and the top edge of each of the respective blanks are provided with narrow bands 13 and 14, respectively, of adhesive tape of the same type as that above referred to. The neckband blanks 11 and 12 are now assembled with the collar top as shown in Fig. 13 and calendered together so that the adhesive tapes 13 and 14 engage the facing ply 3 and the rear ply 5 of the collar top. As illustrated in Figs. 15 and 16, the extensions 9a of the tape 9 project beyond the end edges of the collar top, and after the neckband blanks have been turned as shown in Fig. 14, these extensions 9a are interposed between the ends of the neckband blanks so as to provide reinforcement at the junction of the end of the collar top with the neckband, and to provide additional adhesive material in the ends of the neckband. The end portions of the neckband are now fused together, and the collar is ready for application to a shirt body, the free margins 11a and 12a of the blanks 11 and 12 being folded, as shown in Fig. 14, to provide a finish. If the collar is to be a detached collar, these folded edges may be united in any desired manner, for example by an interposed adhesive tape or by stitching as may be preferred.

In Fig. 17 a simple lapped seam is illustrated, wherein two pieces of fabric 15 and 16 are arranged with their margins in overlapping relation with an adhesive tape 17 interposed between them. This tape is of the type above referred to, and the parts 15 and 16 are permanently and flexibly united by subjecting their overlapped portions with the interposed adhesive to heat and pressure. The pressure applied in forming these seams may be that of a hydraulic press, the press plates being heated electrically or otherwise, but instead of using electrically heated plates, the fusing of the adhesive tape may, for example, be accomplished by electronic high frequency heating; by infra red radiant heating; or by gas heating, and, instead of press platens, rollers may be substituted to provide the desired pressure.

In Fig. 18 there is illustrated a lock or box seam uniting two pieces 23 and 26 of fabric. The piece 23 is doubled at 24 to provide the fold 25, and the piece 26 is doubled at 27 to provide the fold 28. The fold 25 is interposed between the body of the piece 26 and the fold 28, and the fold 28 is interposed between the body of the part 23 and the fold 25. A ribbon or tape 29 of the thermoplastic material is longitudinally folded into a substantially S-shape in transverse section, the parts of this folded tape being interposed as shown in Fig. 18 between the fabric plies, and the parts are subjected to heat and pressure, thus permanently uniting the members 23 and 26 and forming a four-ply seam.

In Fig. 20 another form of seam is illustrated uniting the fabric members 30 and 33. The part 30 is doubled at 31 to form the fold 32, and the part 33 is doubled at 34 to form the fold 35. The folds 32 and 35 are disposed substantially in the same plane or in alignment, and a tape 36 of thermoplastic material is disposed as shown in Fig. 20, one margin being interposed between the part 30 and the fold 35, and the other margin being disposed between the part 33 and the fold 32. The parts are now subjected to heat and

pressure, thus forming a permanent seam to unite the parts.

In Fig. 19 another seam is illustrated wherein the parts 18 and 21 are united by a thermoplastic seam. The part 18 is doubled at 19 to provide the fold 20, and interposed between this fold and the part 21 is a thermoplastic tape 22. The parts are subjected to heat and pressure, thus uniting the members 18 and 21 by a permanent stitchless seam.

As specific examples of the formation of such resin-bonded stitchless seams, the following examples are given:

*Example 1*

A plain lap seam is constructed without any stitching by placing two pieces of fabric together, edge over edge, placing a tape of thermoplastic film between the two pieces of fabric at the overlapping edges and applying heat and pressure to the seam which fuses the resin and thus bonds the seam. The fabric used is a plain-weave cotton broadcloth composed of 40/1 warp and filling yarns weighing 4.0 oz. per yard and having a count of 136 x 60. The thermoplastic film used may be between .002" and .008" thick, preferably .004" thick, and is a milled film of 68 parts vinyl acetate-vinyl chloride copolymer plasticized with 32 parts of di-(2-ethyl hexyl) phthalate. This plasticized resin film is laid along the edge of one piece of fabric and the edge of the other piece of fabric is placed over it. This combination of fabric and resin is then placed between two steel platens, heated by means of electric heating units to a temperature above the softening temperature of the plasticized resin film, approximately 400° F. in this instance, and pressed together by hydraulic pressure of 133 lbs. per square inch. It is found that one second is sufficient time at this temperature and pressure to cause complete fusing of the seam which is then highly resistant to multiple washing and ironing, and can be separated only on application of considerable force, the seam being stronger than the fabric.

The seam as prepared above was subjected to multiple washings, followed by ironing after each wash according to Federal Specifications CCC-T-191a. The seam was examined at periodic intervals, and at the end of 60 such washes was still firmly fused and free from puckering, usually common in sewn seams due to shrinkage of the thread, or discoloration.

*Example 2*

The parts for a three-ply collar are cut in the regular manner with the top ply consisting of a plain-weave cotton fabric of 50/2 warp and 70/3 filling yarns weighing 6.8 oz. per yard and having a count of 110 x 80. The interliner or lining is a plain-weave cotton fabric made of 14/1 warp and filling yarns with a count of 48 x 48 and weighing 5.6 oz. per yarn. The back or rear ply fabric has a count of 136 x 60 and is a plain-weave cotton fabric composed of 40/1 warp and filling yarns, weighing 4 oz. per yarn. The band used is two-ply, the cotton fabric making up the band has a count of 68 x 72, weighs 7.8 oz. per yard and is a plain-weave fabric made of 16/1 warp and filling yarns. The top ply of the band is treated with 12% resin solution composed of 80 parts VYNW (vinyl chloride-vinyl acetate copolymer) and 20 parts of Flexol DOP plasticizer di-(2-ethyl hexyl) phthalate. A tape of thermoplastic resin film  $\frac{1}{8}$ " wide and .004" thick made of 68 parts VYNW and 32 parts of Flexol DOP plasticizer is

calendered or prefused to the bottom and side edges of the back and inner liner on one side of each fabric. The three plies of the collar are then placed together so that the tapes on the 5 backing and the inner liner face the top ply which at this point is between the back and inner liner. The whole collar is then heated under pressure to a temperature slightly above the softening point of the resin for approximately 3 seconds 10 until fused. The points are then trimmed to remove excess cloth and resin and the collar turned inside out, thus placing the three plies in their proper order in the finished collar. The points of the collar are then formed by pulling the end 15 of the collar over a metal plate of the same shape as the collar point, pushing the assembly into a heated die and exerting pressure. The collar is then trimmed along its top edge, and resin tape  $\frac{1}{8}$ " wide is used to fuse the inner liner to the 20 top ply at the top edge. Another resin tape  $\frac{1}{16}$ " wide fuses the inner liner and backing at the top edge and is long enough to extend about  $\frac{1}{2}$  inch beyond the collar at its top edge. This extra tape is utilized later to fuse the plies of the 25 collar band together in part. A  $\frac{1}{16}$ " wide resin tape is next calendered to the neckband portion around the edges and after turning by pressing over a pattern, the shape of the band edge but  $\frac{1}{16}$ " narrower, the bands are then fused to the 30 collar top, thus completing the collar which is now ready for attaching to a shirt body.

Collars as prepared above were subjected to multiple washings and ironings. They were examined at periodic intervals. At the end of 60 washes the collars were still firmly fused and free of wrinkles or puckering usually common in sewn collars due to the shrinkage of the sewing threads. The color of the collars after this number of washes was still good.

40

*Example 3*

A shirt may be constructed without any stitching by making use of the resin bonded seams illustrated in the previous examples. The parts 45 going into the assembly of a shirt are cut in regular manner. The fabric used in the construction of the shirt is a plain-weave cotton fabric of 40/1 warp and filling yarns, weighing 4 ozs. per yard and having a count of 136 x 60. The three-ply collar is made as outlined in Example 2. A thermoplastic resin tape made of 50 68 parts of vinyl chloride-vinyl acetate copolymer plasticized with 32 parts of di-(2-ethyl hexyl) phthalate, said tape being  $\frac{1}{8}$ " wide and .004" thick is used to bond the various parts of the shirt previously requiring sewing. The collar is next attached by fusing the bands of the collar to the shirt, fusing each end and center first. Any extra material is gathered into place near 60 the yoke of the shirt and the entire band is fused to the shirt with heat and pressure.

Shirts as prepared above were subjected to a series of multiple washings and ironings. The shirts were examined at periodic intervals and at the end of 60 washings the seams were still firmly fused. There was also no sign of puckering or wrinkling at the seams which is common with regular sewn seams due to the shrinkage of the sewing thread. The color of the seams remains good through these multiple washings and ironings.

*Example 4*

Any construction fabric may be used but in this case a plain-weave cotton broadcloth was

used, composed of 40/1 warp and filling yarns, weighing 4.0 ozs. per yard and having a count of 136 x 60. The thermoplastic film used was nylon, .004" thick. A thin tape of nylon was placed between fabric plies, as illustrated in Figs. 18, 19 and 20, respectively, and the several combinations of fabric and resin were placed between two steel platens electrically heated to approximately 500° F. (which is slightly above the softening temperature of the nylon film) and pressed together by hydraulic pressure of 133 lbs. per square inch. It was found that one second is sufficient time at this temperature and pressure to cause complete fusing of the seam. Seams as prepared above are highly resistant to multiple washings and ironings, and can not be separated on application of force sufficient to tear the cloth. The seams were examined at periodic intervals and after 60 washings and ironings were still firmly fused and free from puckering, usually common in seams due to the shrinkage of the sewing thread. There is also no unfavorable color developed.

While certain embodiments of the invention have thus been described and illustrated, it is to be understood that the invention is broadly inclusive of any and all applications of the basic principle herein disclosed and which fall within the terms of the appended claims.

We claim:

1. A shirt collar in which the shrinkage and fabric puckering, heretofore due to stitching by thread, is prevented, which comprises a collar top portion having a plurality of superposed layers and a neckband portion also formed of a plurality of layers, the neckband portion overlapping along an edge thereof with an edge of said top portion, a paper thin ribbon of a freely flexible, thermoplastic resin, disposed between said layers of each portion along their free marginal edges and also between abutting and slightly overlapping marginal edges of said portions, said ribbon being adherent to and uniting the layers and portions with which it is in contact to provide alone adequate connection between them in lieu of stitching.

2. A shirt collar in which the shrinkage and fabric puckering, heretofore due to the thread stitching in the collar, is substantially reduced, which comprises a collar top formed of a facing layer, a lining layer, and a back layer, all three layers being superposed face to face and having four marginal edges, a narrow, paper thin, freely flexible, ribbon of thermoplastic resin disposed between the lining layer and the facing and back layers along three corresponding and meeting marginal edges thereof, the neckband being formed of fabric layers disposed in face to face, aligned relation, a corresponding marginal edge

of each of said neckband layers being disposed in overlapping relation with fourth marginal edge of the assembled collar top layers, a narrow, paper thin freely flexible ribbon of thermoplastic resin also disposed between the neckband layers and the top layers at said overlap, said resin being adherent to the face surfaces of the fabrics of the layers engaged thereby but not substantially penetrating to the opposite faces of the layers, whereby the collar is a complete unit requiring no stitching.

3. In the manufacture of a shirt collar of the type having a collar top portion and a neckband portion where each portion is formed of a plurality of layers superposed face to face and the layers of the neckband portion have corresponding marginal edges overlapping with a marginal edge of the assembled collar top layers, that improvement for substantially eliminating collar shrinkage and fabric puckering heretofore due to shrinkage of the stitching by which the layers were connected in each portion and the portions connected together, which comprises the steps of interposing between the superposed layers of each of said portions bordering their free marginal edges and also between the overlapping marginal edges of the assembled top portion and neckband portion, a narrow, paper thin, freely flexible thermoplastic resin, leaving the interior of the superposed layers free of said resin, and ironing assembled layers to soften the interposed resin ribbon and cause it to adhere to the fabrics of the layers engaged thereby without penetration to the opposite faces of those layers.

EDWARD C. PFEFFER, JR.  
LAURENCE M. MILLER.

#### REFERENCES CITED

40 The following references are of record in the file of this patent:

#### UNITED STATES PATENTS

| Number    | Name       | Date          |
|-----------|------------|---------------|
| 2,299,982 | Harrison   | Oct. 27, 1942 |
| 1,673,573 | Loomis     | June 12, 1928 |
| 1,830,639 | Caunitz    | Nov. 3, 1931  |
| 2,087,480 | Pitman     | July 20, 1937 |
| 2,103,492 | Roberson   | Dec. 28, 1937 |
| 265,497   | Hawley     | Oct. 3, 1882  |
| 2,120,458 | Bodie      | June 14, 1938 |
| 2,283,698 | Redman     | May 19, 1942  |
| 2,335,159 | Salfisberg | Nov. 23, 1943 |
| 2,364,903 | Howard     | Dec. 12, 1944 |

#### FOREIGN PATENTS

| Number  | Country       | Date          |
|---------|---------------|---------------|
| 474,598 | Great Britain | Oct. 29, 1937 |
| 444,012 | Great Britain | Mar. 11, 1936 |